

# UNITED STATES PATENT OFFICE.

ANTON LEDERER, OF NEAR VIENNA, AUSTRIA-HUNGARY.

## MANUFACTURE OF FILAMENTS OF TUNGSTEN OR MOLYBDENUM FOR ELECTRIC INCANDESCENCE LAMPS.

1,071,325.

Specification of Letters Patent. Patented Aug. 26, 1913.

No Drawing.

Application filed April 24, 1906. Serial No. 313,485.

*To all whom it may concern:*

Be it known that I, ANTON LEDERER, a subject of Austria-Hungary, residing at No. 83 Atzgersdorf, near Vienna, in the Province of Lower Austria and State of Austria-Hungary, have invented new and useful Improvements in the Manufacture of Filaments of Tungsten or Molybdenum for Electric Incandescence Lamps, of which the following is a specification.

My invention relates to a process for making pure tungsten filaments or wires for incandescent electric lamps, whereby the disadvantages and the troublesome conditions of the known processes such as denitration, heating to incandescence in steam and hydrogen, and equalizing the filaments, are completely eliminated and the simple and rapid manufacture of the metal filaments is insured.

In order to make incandescent electric lamp filaments according to my invention, a certain oxygen compound of the metal, namely tungsten dioxid, is mixed with one or more organic agglutinants, such as an ammoniacal solution of casein, a solution of isinglass, levulose or gum, and the mixture is worked up into a plastic mass, which is then pressed into the form of threads in the usual manner. The latter are allowed to dry, and they are then subjected to dry distillation in the absence of air. During this dry distillation the carbon contained in the organic agglutinant reacts with the oxygen of the tungsten dioxid, and the reduced particles of metal consolidate with a dense, coherent and elastic filament. In order to completely eliminate the carbon of the agglutinant, I proportion the quantity of agglutinant in such a manner that the carbon contained in it is practically chemically equivalent to the amount of oxygen in the dioxid. While various materials may be used as an agglutinant I have found that the ammoniacal solution of casein is peculiarly well adapted to the purpose, as its binding qualities are great and usually a smaller quantity of casein may be used than in the case of any other binder. In general it is desirable that the amount of binding material used shall be as small as possible. I find that the elimination of the carbon and the proper consolidation of the particles of the reduced metal into a dense and elastic filament depend to a large extent upon the

proper conditions under which the process is conducted. In order to obtain the best results the temperature should be around 1200 degrees and the air should be evacuated from the vessel in which the filaments are located as completely as possible. Under these conditions I obtain a dense, coherent and elastic metallic filament, which consists of practically pure tungsten metal and which only contains such small amounts of carbon, that the latter can be considered completely eliminated for practical purposes. The filaments thus obtained are then heated to incandescence in absence of air by passing through them an electric current, for the purpose of eliminating any oxid they may still contain.

It is obvious that it is very difficult in practice to so proportion the carbon of the binder to the oxygen of the tungsten dioxid that they are absolutely chemically equivalent. For this reason I prefer to add a little excess of oxid, which excess I volatilize by the heat of the electric current. As my filaments are already practically completed after the dry distillation process, they are very good conductors of electricity. I therefore do not heat them up gradually to a very high temperature, but subject them at once to a high heat. If the proportion of carbon to the metallic oxid should be in excess, a filament consisting of metal and metal carbid is obtained. This has a much higher electrical resistance than that of a pure metal filament, and if heated to incandescence, will scatter the carbon contained in it owing to electrolytical dissociation. The carbon thus eliminated from the filament deposit only the inner surface of the lamp bulb and blackens it. It is obvious, therefore, that I do not aim at producing any metallic carbids, and that it is preferable for me to use a slight excess of oxid.

The filament obtained by my process has a shining surface of metallic luster and chemical analysis proves that the filament consists of pure metal.

What I claim as my invention is:

1. In the process of manufacturing pure metallic filaments for incandescent electric lamps, a paste for squirting the raw filaments composed of an oxygen compound of a refractory metal and an agglutinant consisting of an ammoniacal solution of casein.
2. In the process of manufacturing pure

tungsten filaments for incandescent electric lamps, a paste for squirting the raw filaments composed of an oxygen compound of tungsten and an agglutinant consisting of 5 an ammoniacal solution of casein.

3. In the process of manufacturing pure tungsten filaments for incandescent lamps, a paste for squirting the raw filaments composed of tungsten dioxid and an agglutinant 10 consisting of an ammoniacal solution of casein.

4. In the process of manufacturing pure tungsten filaments for incandescent electric lamps, a paste for squirting the raw filaments composed of tungsten dioxid and a 15 sufficient amount of an agglutinant consisting of an ammoniacal solution of casein, so that the carbon of the agglutinant is not in excess of the amount chemically equivalent 20 to the oxygen of the tungsten dioxid.

5. The process of manufacturing filaments for incandescent electric lamps, which

consists in preparing a paste containing a quantity of tungsten dioxid and a sufficient amount of organic agglutinant composed 25 of an ammoniacal solution of casein, so that the carbon contained in it is not in excess of the amount chemically equivalent to the oxygen of the dioxid, forming threads from the plastic mass thus prepared in the usual manner, and subjecting the same to dry distillation, thereby converting the carbon of the agglutinant into carbon monoxid or dioxid, reducing the tungsten dioxid to metallic tungsten and consolidating the particles of reduced metal into a dense and coherent filament.

In testimony whereof I have signed my name to this specification in the presence of two subscribing witnesses.

ANTON LEDERER.

Witnesses:

JOHANN LUX,  
ALVESTO S. HOGUE.